

# United States Patent Office

2,900,288

Patented Aug. 18, 1959

1

2,900,288

## PROCESS FOR HEAT-TREATING A BEARING ALLOY

Erich Pelzel, Stolberg, Germany, assignor to Vereinigte Österreichische Eisen- und Stahlwerke Aktiengesellschaft, Linz (Danube), Austria, a firm

No Drawing. Application July 5, 1956  
Serial No. 595,835

Claims priority, application Austria February 9, 1952

2 Claims. (Cl. 148—13)

The invention relates to an aluminum-zinc-copper alloy, which is particularly suitable for replacing the expensive bronzes containing copper and zinc which have previously been used in most cases as a bearing alloy. The invention relates also to a process for heat-treating the bearing members made of that alloy.

The present application is a continuation-in-part of the copending U.S. patent application Ser. No. 334,973 filed February 3, 1953, now abandoned.

Many alloys are known which consist of aluminum and copper, balance zinc. Previously, however, such alloys have been used only in single cases in bearings. For this purpose not only the generally desired higher characteristics as regards tensile strength, elongation and Brinell hardness are to be taken into consideration but also the internal structure and the adherence of oil films on the bearing surface. In that respect too bronzes are preferable to alloys of zinc, aluminum and copper.

In the co-pending application mentioned hereinbefore, an alloy was proposed for bearing purposes which contains 30–66% of aluminum, copper to the amount of at least one sixth and at most one fourth of the actual aluminum content, and the balance of zinc.

The general technological properties of such alloys are satisfactory but it has been found in experiments that in certain marginal regions of the aluminum content disadvantages occur which cannot be tolerated where the alloy is used for bearing bushings.

It has been found that the disintegration of the structure and resultant changes in volume increase as the content of aluminum is reduced. For instance, in an alloy consisting of 30% aluminum, 5% copper, balance zinc, a dimensional change of 0.1–0.2% will result after a storage time of one month. Such a change is not tolerable for bearing bushings because such a shrinkage will obstruct the running of the shaft. Tests with alloys having a higher content of aluminum have shown that these detrimental shrinkage properties do no longer occur in alloys with 35% aluminum, 6.5% copper and 58.5% zinc. As a result, it is apparent that the aluminum content should not be less than 35%.

In further tests it has been shown that the upper limit of the aluminum content is also significant for bearing alloys because this upper limit is of special influence on the structure of the bearing metal. In that respect the interrelations are of a somewhat complex nature, as will become apparent from the following discussion.

When the alloys are being processed with the usual melting and pouring equipment a certain contamination of the alloy by iron cannot be avoided. That contamination has proved to be tolerable when the iron content of low-aluminum alloys does not exceed 0.3%. Micro-photographs of such alloys reveal precipitates consisting of crystals of iron and zinc in the form of small needles, which are not disturbing.

With higher contents of aluminum, particularly up to the limit of 66% stated in the co-pending application

2

mentioned hereinbefore, it was found that the precipitation of iron and zinc crystals increases disproportionately, i.e., by a multiple amount, compared to alloys having a low aluminum content. The explanation found for this phenomenon resides in that with a high aluminum content a ternary field is entered wherein complex aluminum and iron silicon compounds are formed.

These differences depending on the aluminum content appear to be due to the following facts.

10 Where the aluminum content and consequently also the silicon content is small, the affinity of iron and zinc prevails so that the said fine needlelike iron and zinc crystals are formed, wherein one part of iron combines with about 9 parts of zinc. In high-aluminum alloys, having a high silicon content, the affinity relations are changed. One part of iron combines with about twice that amount of silicon and seven times that amount of aluminum to form a ternary crystal, which is voluminous owing to the high share of the lightweight aluminum.

20 That process is promoted by the fact that the rate of crystallization of that ternary phase is so high that a relatively small number of coarse crystals are formed instead of the aforementioned numerous fine needles.

25 The commercially pure aluminum, which is to be used for foundry purposes for economic reasons, contains always impurities up to 0.5% silicon. For this reason the detrimental content of silicon in the alloy can be kept down only by preventing the content of aluminum for exceeding a tolerable amount.

The tests made have shown that the undesired coarse ternary crystals begin to occur with an aluminum content of 50%, i.e. with a silicon content of about 0.25% if the contamination of the aluminum by silicon amounts

30 to 0.5%. In order to avoid the disadvantages set forth hereinbefore, residing in undesired dimensional changes and the formation of coarse ternary crystals, therefore, the teaching given in the co-pending application mentioned hereinbefore must be modified so that the aluminum content of the bearing alloy amounts to 35–50%, the copper content amounts at least to one sixth and at most to one fourth of the actual aluminum content, and the balance consists of zinc.

35 The range of alloys possible is limited by the series of alloys having the lowest copper content (copper content=1/6 aluminum) and by the series of alloys having the highest copper content (copper content=1/4 aluminum content).

40 The series of alloys having the lowest copper content is:

| Al          | 35   | 40   | 45   | 50   |
|-------------|------|------|------|------|
| Cu(=1/6 Al) | 5.8  | 6.7  | 7.5  | 8.3  |
| Zn          | 59.2 | 53.3 | 47.5 | 41.7 |

45 The series of alloys having the highest copper content is:

| Al          | 35   | 40 | 45   | 50   |
|-------------|------|----|------|------|
| Cu(=1/6 Al) | 8.8  | 10 | 11.2 | 12.5 |
| Zn          | 56.2 | 50 | 43.8 | 37.5 |

50 These alloys are processed to form bearing by casting, or casting and hot-working, or casting and cold-working. In this manner sleeves, half-brasses or bushings are made. The technological characteristics are:

55 Specific gravity: 4.5 to 4.0  
Tensile strength: 30–35 kg./sq. mm.  
60 Elongation: 3–6%  
Brinell hardness number: 100–140 kg./sq. mm.

65 The shaped bearing members may be subjected to an

after treatment to improve the properties of the bearing alloy. That aftertreatment is performed, e.g., by heating the shaped parts to a temperature of 100-280 deg. C. The duration of the heat treatment is at least three hours, preferably 24-48 hours. The effect achieved by the aftertreatment is surprising.

Whereas without heat treatment the elongation is 3-6%, it increases after the treatment to 5-10%. The strength and hardness remain substantially unchanged.

The improvement of the properties by the aftertreatment is explained by a change in internal structure. In the range of concentrations stated the zinc-aluminum-copper alloys consist of a ternary phase and aluminum-zinc mixed crystal. The treatment according to the invention leads to a partly eutectoid disintegration of the ternary compound, whereby the structure is refined and incorporated zinc mixed crystals occur. In connection therewith, the running characteristics of the alloy and its suitability as a bearing material are changed in the desired sense.

The metals used for the production of the alloys need not be perfectly pure. Since it has been proved that a lead content up to 1.5% does not adversely affect the running properties, nor the corrosion behavior, ordinary zinc of commercial purity may be used to advantage as an alloying constituent.

*Example 1*

From an alloy containing 35% aluminum, 7.5% copper, balance commercially pure zinc, a bearing sleeve is made by casting and heat-treated at 250 deg. C. for 24 hours. The strength is 32 kg./sq. mm., the elongation 10%, the Brinell hardness number 120 kg./sq. mm. When the bearing was loaded with 50 kg./sq. cm. a maximum temperature rise of 60 deg. C. was observed.

30  
15  
20  
25

*Example 2*

From an alloy containing 40% aluminum, 8% copper, and the balance of commercially pure zinc, a bearing sleeve is made by casting and is heat-treated at 250 deg. C. for 24 hours. The strength is 32.5 kg./sq. mm. the elongation 5%, the Brinell hardness number 108 kg./sq. mm. When the bearing was loaded with 50 kg./sq. cm., a maximum temperature rise of 70 deg. C. was observed.

5  
10  
15  
20  
25

I claim:

1. A method of producing an aluminum-zinc-copper alloy for bearing purposes comprising the steps of: producing a composition alloy of 35 to 50% Al, 5.8 to 8.3% Cu, 0 to 0.3% Fe, 0 to 0.25% Si, and 59.2 to 41.15% of Zn; of shaping said alloy, and of heat-treating said alloy at temperatures from 100 to 280° C. for a time from 24 to 48 hours.
2. A method of producing an aluminum-zinc-copper alloy comprising the steps of producing an alloy composition of 35 to 50% Al, 8.8 to 12.5% Cu, 0 to 0.3% Fe, 0 to 0.25% Si, and 56.2 to 36.95% of Zn, and heat-treating said alloy at temperatures from 100 to 280° C. for a period from 24 to 48 hours.

25  
20  
15  
10  
5  
2. References Cited in the file of this patent

UNITED STATES PATENTS

- 1,212,374 McAdams \_\_\_\_\_ Jan. 16, 1917  
2,388,563 Nock et al. \_\_\_\_\_ Nov. 6, 1945

FOREIGN PATENTS

- 448,929 Great Britain \_\_\_\_\_ June 17, 1936.

OTHER REFERENCES

- 1948 Metals Handbook, page 1244.